

1

3,728,169

## ENCAPSULATION OF NITRONIUM PERCHLORATE EMPLOYING AMMONIA TO FORM AMMONIUM PERCHLORATE

James P. Diebold, China Lake, Calif., assignor to the United States of America as represented by the Secretary of the Navy  
No Drawing. Filed Mar. 18, 1963, Ser. No. 266,105  
Int. Cl. C06d 5/06

U.S. CL. 149—5

5 Claims

The invention described herein may be manufactured and used by or for the Government of the United States of America for governmental purposes without the payment of any royalties thereon or therefor.

The present invention relates to a process for the encapsulation of nitronium perchlorate particles.

Nitronium perchlorate is an extremely reactive substance. Studies on the use of this material as an oxidizer in propellants show that theoretically a specific impulse of near 300 seconds is possible. However, because of its highly reactive nature, passivation in one form or another

2

volving the passing of dry ammonia gas over particles of nitronium perchlorate.

An object of the present invention is to provide an encapsulating technique for rendering high energy solid fuels and oxidizers inert to each other and to the binder material until such time as the system is ignited.

Another object is to provide a method for encapsulating nitronium perchlorate for use in the propellant field.

A further object is to provide nitronium perchlorate particles having continuous coatings which isolate the nitronium perchlorate from the propellant binder.

Other objects and advantages of this invention will become readily appreciated as the same become better understood by reference to the detailed description.

The present invention is essentially concerned with encapsulation of nitronium perchlorate (NP) with ammonium perchlorate (AP) by a reaction process comprising the passing of dry ammonia gas (NH<sub>3</sub>) over particles of nitronium perchlorate whereby the ammonia reacts with the nitronium perchlorate to form ammonium perchlorate on the surface of each particle.

A simplified diagram of the process is as follows:



is necessary. Literature surveys show that the work in the past toward passivation of nitronium perchlorate has been directed toward encapsulation with an inert plastic binder or with an aluminum coating. These passivation techniques have not proved entirely satisfactory. One disadvantage is that there is a decrease in theoretical specific impulse ( $I_{sp}$ ) due to the use of essentially inert organic encapsulating compounds. Other disadvantages include a non-continuous coating which does not effect complete protection of the nitronium perchlorate from the binder at ambient conditions, a lack of long-term protection with a reasonable coating thickness, and a lack of protection from water vapor which decomposes the nitronium perchlorate. The general purpose of this invention is to provide a method of encapsulation which embraces all the advantages of similarly employed methods and possesses none of the aforementioned disadvantages. To attain this, the present invention contemplates a unique process in

55 The equipment used consisted primarily of glassware connected by rubber hoses. To control the flow rates of the helium (used as an inert diluent) and ammonia, micrometer valves were installed and calibrated. Later it was found that with these valves one could not control the flow rates as accurately as was desired, and rotameters were 60 installed to augment the flow control. Due to the exothermic nature of the reaction, the incoming gases and the reaction vessel (a glass U-tube) were cooled by ice baths. The helium was found to be wet and it was necessary to install a drying unit filled with molecular sieves.

65 A series of experiments were conducted using nitronium perchlorate pellets weighing about 3 milligrams each and ammonia gas ranging in concentration from about 5% to 60%. The initial reaction temperatures were maintained at about 34° F., but was also found that the reaction would occur at initially ambient conditions. The following examples are illustrative of the process above.

**3**  
**EXAMPLE I**

4 pellets of nitronium perchlorate weighing about 12 milligrams were placed in the reactor (a glass U-tube) which was cooled by an ice bath. A 60% concentration of ammonia gas was passed over the pellets. The flowrate for the ammonia was about 9.6 cc. per second, and the dried helium about 6.2 cc. per second through the  $\frac{3}{8}$  inch diameter glass tubing reactor. The reaction was continued for about 8 minutes at 34° F. The pellets were then tested for encapsulation by casting them in a polyurethane binder. This binder is not compatible with nitronium perchlorate and is, in fact, incompatible with some forms of plastic-encapsulated nitronium perchlorate. One pellet of this experiment was coated and found to be compatible with the binder. Two of the pellets were completely reacted with the ammonia and one pellet was lost during the reaction when it dissolved.

**EXAMPLE II**

Following the same procedure outlined above three nitronium perchlorate pellets were treated with an 8% concentration of ammonia diluted with dry helium. The flowrate of the gases was controlled to about 6 cc. per second for 15 minutes at an initial reaction temperature of 34° F. One pellet was completely encapsulated and did not react with the polyurethane binder.

It is postulated that the process may be represented by the following multistep equation:



It was found that pellets of the same run would not necessarily react similarly. Liquid formation was observed during many of these runs. If the pellets were to have been wetted during the first stage of the process before the ammonia had diffused throughout the pellet, then this liquid would act as a barrier to further ammonia penetration. This apparently would limit the reaction to the surface of the pellet to form the desired coating.

The liquid formed by the overall reaction was the subject of much theorizing. In some experiments this liquid did not necessarily collect entirely around all the pellets. There was observed occasional condensation of the liquid down-stream from the pellets. This liquid would eventually solidify into a white material. The white material was observed to be inert with respect to the binder. The most plausible explanation for this phenomena is that the liquid formed was anhydrous perchloric acid ( $\text{HClO}_4$ ) and nitric acid ( $\text{HNO}_3$ ). The solidification process would then be the reaction of the basic ammonia ( $\text{NH}_3$ ) with the acids, shown in Equation 3 above.

Since it appears that a multistep process is probable, if conditions are varied such that one reaction is favored over another, the resultant products will also be varied. It was observed that Equations 1 and 2 above, were favored at the higher ammonia ( $\text{NH}_3$ ) concentrations as evidenced by a considerable liquid formation. At lower concentrations of ammonia (see Example II) Equation 3 was favored because there was no observable liquid formation. This would indicate that the liquid was reacting with the ammonia at a rate comparable to the rate of formation of the liquid.

It should be noted that nitronium perchlorate and ammonium perchlorate have different crystal structures and therefore a disordered crystal may result. A disordered crystal would have different decomposition characteristics than those of the pure substances. It is thought that ammonium perchlorate was possibly produced in the cubic form by this reaction, as Differential Thermal Analysis did not reveal the ammonium perchlorate phase change from rhombic to cubic.

**4**

The variations in results of some of the experiments carried out in trying to perfect the present process could be due to varying porosity, possible variation of composition on the pellets, and local concentration of the ammonia in the gas stream. If the pellets were porous, ammonia would have an opportunity to diffuse throughout the pellet causing complete reaction with the nitronium perchlorate.

A slight variation in the procedure described in Examples I and II is proposed below:

**EXAMPLE III**

After placing the nitronium pellets in the reactor the first step would be to pass a high concentration of ammonia (10% to 60%) over the pellets to form a liquid (anhydrous perchloric acid). This would be followed by a helium purge to rid the system of ammonia and reaction products and to reduce the temperature of the pellets. Then a low concentration of ammonia (less than 5%) would be passed over the pellets to react with the liquid on the surface forming the desired ammonium perchlorate coating. This reaction may be represented by the following equation:



In another series of experiments a crystalline form of nitronium perchlorate was used which had a particle size of 3 to 5 microns. The reaction time was about 15 minutes at about 34° F. Using a concentration of 40% ammonia, some of the nitronium crystals reacted to form a liquid which cemented the remaining crystals together to form a solid mass. In the concentration range between 5% and 40% reaction took place which did not form a solid mass. However, there was observed a definite trend of less agglomeration with lower ammonia concentration. Using 4% ammonia, there was no obvious physical or chemical change in the material. At ice bath temperatures, 4.7% ammonia appears to be about the lowest concentration that will promote a reaction. The observation of the effect of varying ammonia concentrations are shown in Table I below:

45 TABLE I.—EFFECT OF  $\text{NH}_3$  CONCENTRATION  
(15 minute reaction time, using 3-5 micron NP crystals)

| Percent $\text{NH}_3$ in He stream | Appearance of product in moist atmosphere |
|------------------------------------|-------------------------------------------|
| 0.7                                | Fumed. <sup>1</sup>                       |
| 1.6                                | Do.                                       |
| 3                                  | Do.                                       |
| 4                                  | Do.                                       |
| 4.7                                | Did not fume.                             |
| 5                                  | Fumed slightly (later did not fume).      |
| 5                                  | Did not fume.                             |
| 5                                  | Do.                                       |
| 6                                  | Do.                                       |
| 8                                  | Do.                                       |
| 10                                 | Do.                                       |
| 20                                 | Do.                                       |
| 30                                 | Do.                                       |
| 40                                 | Did not fume (agglomerated).              |
| 50                                 | Do.                                       |

<sup>1</sup> Fuming indicates presence of  $\text{NO}_2\text{ClO}_4$ .

65 In order to determine the conditions favorable for the desired reaction in which the coating was formed, the solid products were analyzed. The qualitative tests showed that ammonium nitrate and ammonium perchlorate are possible reaction products as shown in Equation 3 herein. Ammonium nitrate may not necessarily be present as the  $\text{NO}_2^+$  ion of nitronium perchlorate would be analyzed as  $\text{NO}_3^-$ .

70 This invention is concerned with the problem of obtaining a coating on the surface of the nitronium perchlorate. It was observed that in many instances the ammonia had reacted with all of the nitronium perchlorate in the particle which was thereby rendered inert with respect to the binder. It was found during the process of

casting the pellets coated in Example I above into the binder, that when some of the pellets were prodded, the coating was fractured exposing a mushy interior indicating the reactions of  $\text{NH}_3$  with most of the NP in the pellet.

Obviously, many modifications and variations of the present invention are possible in the light of the above teachings. It is therefore to be understood that within the scope of the appended claims the invention may be practiced otherwise than as specifically described.

What is claimed is:

1. A process for encapsulating nitronium perchlorate comprising the step of

flowing ammonia diluted with an inert gas over nitronium perchlorate particles.

2. A process for coating nitronium perchlorate particles with ammonium perchlorate which comprises

(a) flowing about a 60% concentration ammonia gas over nitronium perchlorate particles until said particles are wetted; and

(b) continuing the flow of ammonia over said particles for about 8 minutes at about 34° F. until the wetting liquid has disappeared around each particle.

3. A process for coating nitronium perchlorate with ammonium perchlorate which comprises the following multistep reaction:

- (a)  $\text{NH}_3 + \text{NO}_2\text{ClO}_4 \rightarrow \text{H}_2\text{O} + \text{HClO}_4 + \text{oxides of nitrogen}$   
 (b)  $\text{H}_2\text{O} + \text{NO}_2\text{ClO}_4 \rightarrow \text{HNO}_3 + \text{HClO}_4$   
 (c)  $\text{NH}_3 + \text{HClO}_4 + \text{HNO}_3 \rightarrow \text{NH}_4\text{ClO}_4 + \text{NH}_4\text{NO}_3$   
 (d)  $\text{NH}_4\text{NO}_3 + \text{NO}_2\text{ClO} \rightarrow \text{NH}_4\text{ClO}_4 + \text{oxides of nitrogen}$

5 4. A process for encapsulating nitronium perchlorate particles which comprises

subjecting nitronium perchlorate particles to a continuous flow of ammonia and helium for about 10 minutes at ambient temperature for forming a film of ammonium perchlorate around the particles.

10 5. Particulate nitronium perchlorate coated with ammonium perchlorate.

#### References Cited

#### UNITED STATES PATENTS

- 3,006,743 10/1961 Fox et al. \_\_\_\_\_ 149—19  
 3,535,172 9/1969 Bieber et al. \_\_\_\_\_ 149—7

20 BENJAMIN R. PADGETT, Primary Examiner

U.S. CL. X.R.

117—100 B; 149—19, 75; 423—386, 476